

April 26, 1927.

1,626,276

G. J. ESSELEN, JR

PROTECTING COVERING FOR RUBBER SHEETS

Filed March 29, 1924

*Fig. 1.*



*Fig. 2.*



*Fig. 3.*



INVENTOR

Gustave J. Esselein, Jr.  
by his attorneys  
Byrnes, Stabbins & Parmalee

Patented Apr. 26, 1927.

1,626,276

# UNITED STATES PATENT OFFICE.

GUSTAVUS J. ESSELEN, JR., OF SWAMPSCOTT, MASSACHUSETTS.

## PROTECTING COVERING FOR RUBBER SHEETS.

Application filed March 29, 1924. Serial No. 702,771.

Figure 1 is a perspective view of a portion of a sheet of rubber with the protective covering applied.

Figure 2 is a cross section through the rubber and protective covering, and

Figure 3 is a cross section similar to Figure 2 showing a modification.

The present invention relates to protecting rubber sheets, and more particularly to protecting unvulcanized rubber sheets to keep the sheets from sticking together. The usual material used for this purpose is the so called "holland" made from a strong cotton fabric which is provided with a smooth glaze. This fabric is smooth enough so that it can be stripped from the sticky surface of unvulcanized rubber and is strong enough so as not to readily tear when stripped off. The material, however, is expensive. I have discovered that the paper known to the trade as glassine paper may be employed as a satisfactory and inexpensive substitute for the fabric holland as a protecting coating for sheet rubber. This glassine paper is a stock product and can be easily obtained and may be used without special treatment. This paper is mechanically tough; it has a highly glazed surface which permits it to be readily stripped from the surface of unvulcanized rubber, and has a homogeneous substantially transparent body through which the surface of the rubber is visible for inspection. Glassine paper is made from cellulose pulp which has been mechanically hydrated. It is made by a wet milling process in which the cellulose fibers are subjected to crushing and rubbing in the presence of water. This mechanical action is carried to a point where the cellulose fibers are reduced to a hydrated pulp, from which the glassine paper is made. The sheet formed from the hydrated cellulose pulp is passed in a moist condition between highly polished heater calender rolls under pressure in order to give it a smooth highly glazed surface. The term "glassine paper" is ordinarily employed in the trade to describe a paper having a glass-like or glazed surface and made from mechanically hydrated cellulose pulp, as distinguished from chemically parchmentized papers. Paper is ordinarily chemically parchmentized by passing a sheet of the formed paper through a bath of sulphuric acid which superficially dissolves the surfaces of the sheet, leaving the fibers in the interior of the sheet sub-

stantially unaffected. This chemically parchmentized paper does not have the homogeneous substantially transparent body of glassine paper. The chemical parchmentizing treatment does not produce a glazed surface like that of glassine paper, but on the contrary produces a characteristic uneven cockled surface which it is very difficult, if not impossible, to eliminate by calendering. Moreover, the chemical parchmentizing treatment leaves certain chemical residues in the paper, which, unless the greatest pains are taken to remove them, would have a deleterious effect, in time, on the paper or on rubber in contact with the paper or on both. Suggestions have been made to employ chemically parchmentized paper as a liner for sheet rubber, but if so used it would require special calendering and softening treatment before it could be used at all, whereas glassine paper may be employed without such special treatment.

In Figures 1 and 2 of the drawings is illustrated the rubber sheet with the glassine paper protective coating applied thereto. In these drawings 1 indicates the rubber sheet and 2 the glassine paper protective coating.

While the glassine paper, if made with a moderately heavy body, has sufficient strength to enable it to be stripped from the rubber, it may be combined with a backing of a stronger or heavier bodied paper, such as a kraft paper. The term "kraft" paper is employed in the paper trade to designate certain papers of special quality having unusually tough fiber, the word being adopted from the German word "kraft" which means strength. A composite protecting sheet for rubber may be made from a backing of a heavier paper, such as a kraft paper, and a facing of glassine paper on one or both sides of the backing, and secured thereto by a flexible adhesive such, for example, as a flexible glue made from animal glue, glycerine and water.

In Figure 3 is illustrated diagrammatically the modification of the invention, and in which 1 indicates the rubber sheet, 2 the glassine paper and 3 the backing of kraft paper.

While the preferred embodiment of the present invention has been specifically described it is to be understood that the invention is not limited to all of the details hereinbefore described, but may be otherwise

embodied within the scope of the following claims.

I claim:

1. The combination with a sheet of rubber, of a readily separable protecting sheet of smooth surfaced glassine paper, substantially as described.
2. The combination with a sheet of rubber, of a readily separable protecting sheet of paper made from mechanically hydrated cellulose pulp and having a smooth highly glazed surface which permits it to be readily stripped from the rubber, substantially as described.
3. The combination with a sheet of rubber, of a readily separable protecting sheet of paper having a substantially transparent homogeneous body made from mechanically hydrated cellulose pulp and having a smooth highly glazed surface which permits it to be readily stripped from the rubber, substantially as described.
4. The combination with a sheet of rubber, of a readily separable protecting sheet of paper formed from a hydrated cellulose pulp into a substantially transparent homogeneous sheet and calendered to give it a smooth highly glazed surface which permits it to be readily stripped from the rubber, said paper being employed without chemical parchmentizing treatment or impregnation with softening agents, substantially as described.
5. The combination with a sheet of rubber, of a readily separable protecting sheet of glassine paper having a strengthening backing of a kraft paper, substantially as described. 35
6. The combination with a sheet of rubber, of a readily separable protecting sheet of paper made from mechanically hydrated cellulose pulp and having a highly glazed surface which permits it to be readily stripped from the rubber, and having a strengthening backing of a heavier tough fibered paper, substantially as described. 40 45
7. The combination with a sheet of rubber, of a readily separable protecting sheet of paper made from mechanically hydrated cellulose pulp and having a highly glazed surface which permits it to be readily stripped from the rubber, and having a strengthening backing of a tough fibered stronger paper secured thereto with a flexible adhesive, substantially as described. 50
8. The combination with a sheet of rubber, of a readily separable protecting composite sheet of paper formed of a strengthening paper backing, and a facing on both sides thereof composed of a highly glazed paper made from mechanically hydrated cellulose pulp, substantially as described. 55 60

In testimony whereof I have hereunto set my hand.

GUSTAVUS J. ESSELEN, JR.